

**1**

3,366,482

**PROCESS FOR THE PREPARATION OF SILVER HALIDE EMULSIONS BY THE FLOCCULATION METHOD**

Heinrich Schaller and Walter Anderau, Fribourg, Switzerland, assignors to Ciba Limited, Basel, Switzerland, a Swiss company

No Drawing. Continuation-in-part of application Ser. No. 307,376, Sept. 9, 1963. This application Mar. 7, 1967, Ser. No. 621,117

Claims priority, application Switzerland, Sept. 13, 1962,  
10,850/62  
9 Claims. (Cl. 96—94)

**ABSTRACT OF THE DISCLOSURE**

In the process for the preparation of photographic silver halide emulsions the extraneous soluble salts resulting from the reaction of silver nitrate with water-soluble halides in an aqueous gelatine solution, are removed by flocculation of the silver halide emulsion. The flocculation is carried out at a pH of 3 to 7 and the emulsion starts to flocculate immediately on the addition of the flocculating agent. The flocculating agents are colorless compounds that contain at least one six-membered heterocyclic ring made up of 3 to 4 carbon atoms, at the most one halogen atom being bound to a carbon atom of said heterocyclic ring, at least one aromatic radical, and at least one acidic group imparting solubility in water to the compound. The six-membered heterocyclic ring which may be substituted by at the most one halogen atom, e.g. bromine, but more especially chlorine, may also contain other substituents, under the conditions of this flocculating process, no gelatine derivatives are formed together with the flocculating agents.

Photographic silver halide emulsions of all kinds, especially color emulsions, may be prepared by this process.

**Cross-reference**

This application is a continuation in part of applicants' copending application Serial No. 307,376, filed September 9, 1963, now abandoned the disclosure of which is relied on and incorporated by reference in this application.

**Background**

The present invention relates to a process for the preparation of photographic silver halide emulsions in which the extraneous soluble salts are removed by flocculation of the silver halide.

In the preparation of photographic silver halide emulsions, a water-soluble silver salt, generally silver nitrate, is usually reacted with water-soluble halides in an aqueous gelatine solution. The gelatine/silver halide emulsion thus formed contains water-soluble salts which are by-products of the double decomposition reaction, and these salts have to be removed. The conventional method of removing the salts consists in solidifying the emulsion by cooling, comminuting it, and then washing out the salts with cold water.

Another method, known as the flocculation method,

**2**

consists in precipitating the silver halide and the gelatine or other colloid, separating the supernatant salt solution from the precipitate, and then dispersing the precipitate in a gelatine solution or in some other suitable layer colloid.

5 The flocculation method offers a number of advantages; in particular, it makes possible the preparation of concentrated silver halide emulsions. Various methods of flocculating silver halide emulsions have been proposed, for example, flocculation with an inorganic salt, such as, for example, sodium sulfate. However, a large amount of the inorganic salt is required, and the precipitate has to be removed by washing out. Organic solvents can also be used for bringing about flocculation, but this method is expensive and the precipitates obtained are highly voluminous and still contain a large amount of liquid. It has also been proposed to use the salts of heavy metals as flocculating agents. However, such salts have the disadvantage that they harden the gelatine and the precipitates are very difficult to re-disperse. It has also been suggested that anionic substances such as soaps be used, but in this process residual soap adheres tenaciously to the coagulate and tends to cause cloudiness in the emulsion.

Other methods are based on the use of gelatine derivatives. In the preparation of gelatine derivatives, at pH values of 8 to 11 or more involving reaction times of a few minutes up to 30 minutes however, the reactive amino groups of the gelatine undergo change, thus causing a change in the photographic and colloidiochemical properties of the gelatine. Moreover, gelatine derivatives can only be flocculated at a low pH value, for example, at a pH value of about 3.5. In the case of highly sensitive ammonia emulsions, such as are used in the preparation of X-ray films, this unavoidable depression of the pH value to about 3.5 brings about a loss in sensitivity of the emulsion.

**Detailed description**

The present invention is based on the observation that certain heterocyclic compounds are very suitable as 40 flocculating agents. Accordingly, the present invention provides a process for the preparation of photographic silver halide emulsions by the flocculation method, which comprises flocculating the emulsion at a pH of 3 to 7, and using as a flocculating agent a colorless compound 45 containing

(a) At least one six-membered heterocyclic ring made up of 3 to 4 carbon atoms, at the most one halogen atom being bound to a carbon atom of said heterocyclic ring;  
(b) At least one aromatic radical, and  
50 (c) At least one acidic group imparting water-solubility to the compound, the emulsion starting to flocculate immediately on the addition of the flocculating agent.

The acidic group imparting solubility in water present in a flocculating agent according to the invention may be, 55 for example, a carboxylic acid group or a sulfato group, but is preferably a sulfonic acid group. The said flocculating agent must also contain at least one six-membered heterocyclic ring that contains as ring members either 3 carbon atoms and 3 nitrogen atoms or 4 carbon atoms and 2 nitrogen atoms. This six-membered heterocyclic ring may be substituted by at the most one halogen atom and/

or other substituents. Examples of suitable heterocyclic rings are the pyridazine and pyrimidine rings. Compounds that contain at least one 1:3:5-triazine radical are particularly suitable.

The compound to be used as a flocculating agent in the process of the present invention must contain at least one aromatic radical, advantageously an aromatic radical of the benzene or naphthalene series. The aromatic radical advantageously contains at least one substituent, for example, the group imparting solubility in water, and is advantageously bound to the heterocyclic ring either directly or through a bridge, for example, a sulfur or oxygen atom, or preferably a nitrogen atom.

A 1:3:5-triazine compound may be substituted in, for example, each of the 2 and 4 positions by an aromatic radical of the kind defined. The 6 position may have as a substituent a halogen atom, for example, bromine, but more especially chlorine. Examples of suitable triazine compounds fall within the formula



in which  $R_1$  and  $R'_1$  each represents a benzene or naphthalene radical containing at least one sulfonic acid group and  $Y$  represents a halogen atom. The benzene or naphthalene radical may contain another substituent, for example, a further sulfonic acid group, a carboxylic acid group, an alkyl group such as a methyl or ethyl group, an alkoxy group such as a methoxy or ethoxy group, a halogen atom such as chlorine, fluorine or bromine, or a group of more complex structure, for example, a trifluoromethyl group or a sulfonic acid amide group.

In general, the efficacy of the flocculating agent is enhanced by increasing the size of the molecule. Efficacy is further increased by the incorporation of naphthalene radicals, such radicals advantageously being 1- or 2-amino-naphthalene-mono-, di- or tri-sulfonic acids, which thus produce, for example, compounds of the formula



in which  $R_2$  and  $R'_2$  each represents a naphthalene radical containing at least one sulfonic acid group.

A process which comprises condensing a condensation product of equimolecular proportions of cyanuric chloride and an aromatic amino-sulfonic acid, especially an aminonaphthalene disulfonic acid, with an aliphatic or aromatic diamine in a molar ratio of 1:1 results in the formation of a flocculating agent that contains a free amino group. It has been observed that such amino compounds are highly effective at pH values around 5 and 6.

These amino compounds may also be further condensed with a suitable reactive halogen compound, for example, with a condensation product of equimolecular proportions of cyanuric chloride and an aromatic sulfonic acid already mentioned. In such manner there are obtained, for example, flocculating agents that correspond to the formula



in which  $R_2$  and  $R'_2$  each represents a naphthalene radical containing at least one sulfonic acid group, and  $Z$  represents a bridge member. Symmetrical compounds of the kind defined may also be prepared by condensing cyanuric

chloride with aminonaphthalene sulfonic acids and diamines in a molar ratio of 2:2:1, respectively.

It is also possible to join together at the amino groups two identical molecules or two different molecules of the above-mentioned compounds containing a free amino group and formed from one molecule each of an aromatic amino sulfonic acid, cyanuric chloride and a diamine, the link being made through suitable bridge members. There may also be used triazine compounds that no longer contain a halogen atom bonded to the triazine ring. These are obtained, for example, when the last halogen atom in compounds of the kind defined above is exchanged for HO, H<sub>2</sub>N or H<sub>2</sub>C—O groups or substituted amino groups.

The following compounds may be used as starting materials for the preparation of flocculating agents having a composition given above:

- 1-aminobenzene-2-, -3- or -4-sulfonic acid,  
amino-methylbenzene sulfonic acids,  
amino-chlorobenzene sulfonic acids,  
20 amino-methoxybenzene sulfonic acids,  
1-aminonaphthalene-4-, -5-, -6- or -7-sulfonic acid,  
2-aminonaphthalene-4-, -5-, -6- or -7-sulfonic acid,  
1-aminonaphthalene-2:5-, -2:6-, -3:8-, -4:6-, -4:7-,  
-4:8-, -5:7- or -6:8-disulfonic acid,  
25 2-aminonaphthalene-1:7-, -3:6-, -3:7-, -4:7- or -5:7-disul-  
fonic acid, but more especially,  
2-aminonaphthalene-4:8-disulfonic acid,  
1-aminonaphthalene-2:4:6-, -3:5:7-, -3:6:8- or -4:6:8-  
trisulfonic acid,  
30 aliphatic diamines of the formula



in which  $n$  represents an integer of a value not greater than 5,

- 35 1:4-diaminobenzene,  
 1:3-diaminobenzene-4-sulfonic acid,  
 1:3-diaminobenzene-4- or -5-carboxylic acid,  
 4:4'-diaminodiphenyl,  
 4:4'-diaminodiphenyl-2:2'-disulfonic acid,  
 40 4:4'-diaminodiphenyl-3:3'-dicarboxylic acid,  
 3:3'-dicarboxymethoxy-4:4'-diaminodiphenyl and  
 1:5-diaminobenzene-3:7-disulfonic acid.

Some of the flocculating agents in accordance with the invention may be prepared by conventional methods. The following are a number of triazine compounds in accordance with the invention. (The triazine radical of the formula



is simplified as follows:







The compounds given above may be used as flocculating agents in the usual manner. Depending on their constitution, small amounts of these agents bring about good and immediate flocculation at a moderately raised temperature and at pH values in the range of from 3 to 7. It has been observed that, in the short time between the flocculation and any washing out operation, the flocculating agents of the invention do not chemically react with gelatine forming gelatine derivatives and do not cause hardening of the gelatine when used in the small amounts required, even when flocculation is carried out with halogen triazine compounds which are reactive.

In general, flocculation is advantageously brought about by adding an aqueous solution of the flocculating agent to the emulsion, and then adjusting the pH value of the emulsion to the requisite value. However, it is also possible to adjust the pH value first and then add the flocculating agent. The silver halide precipitates along with the gelatine or other colloid in the form of fine granules and settles out very quickly. The precipitate contains only a very small amount of water so that it is generally not necessary to wash it out further. Should it appear necessary, however, the precipitate may be washed out once or several times with cold water; if necessary, the pH value can be adjusted to a suitable value. The pH value for

55 flocculation, is in the range of from 3 to 7, preferably 3 to 5, and the requisite amount of flocculating agent, for example, 10 to 200% (calculated on the dry weight of the gelatine or other colloid) in the form of a dilute aqueous solution, depend not only on the flocculating agent itself, but also on the gelatine or other colloid concentration of the emulsion, the salt content, and other factors. The temperature at which flocculation is carried out has no great influence; it is advantageously within the range of 30 to 50° C., and it should always be such that no substantial amounts of gelatine or of another colloid react with the flocculating agent, in so far as the latter contains reactive groups.

65 Photographic silver halide emulsions of all kinds may be prepared by the process of the invention, especially color materials that contain either dyestuff components for color development or image dyestuffs for the silver dyestuff bleaching process.

70 The following examples illustrate the invention, the parts and percentages being by weight.

#### EXAMPLE 1

A solution of 60 grams of silver nitrate in 600 milliliters of water is added in a period of 15 minutes at 75 50° C. to solution of 8 grams of gelatine, 44 grams of

potassium bromide and 1 gram of potassium iodide in 600 milliliters of water. The mixture is allowed to mature for 10 minutes at 50° C. and is then cooled to 40° C. 30 milliliters of a 5% aqueous solution of the compound of Formula 20 is then added, and the pH of the emulsion is adjusted to 4.5 to 5.0 by the addition of citric acid. The nature of the acid used has no influence on the flocculation process; acetic acid, hydrochloric acid, sulfuric acid or any other acid with a sufficient degree of acidity can also be used. The silver halide precipitates at once along with the gelatine in the form of finely divided granules and settles out very quickly. The supernatant salt solution is decanted off. A solution of 120 grams of gelatine in 1400 milliliters of water and having a temperature of 40° C. is added to the granules, and the pH value is adjusted to 7.0 by the addition of aqueous sodium hydroxide solution. The silver halide is redispersed by stirring for 10 to 20 minutes at 40° C., and the emulsion is allowed to mature to optimum sensitivity in a known manner at 50 to 55° C.

Solutions of the compounds listed in the following Table I may also be used to bring about flocculation of silver halide/gelatine emulsions by the above method instead of a solution of the compound of Formula 20. The amounts required, concentrations and pH values are also listed. All compounds yield emulsions having the same photographic properties.

TABLE I

| Formula No. | Amount, ml. of the solution | Concentration, percent of the solution | pH value at which flocculation is effected |
|-------------|-----------------------------|----------------------------------------|--------------------------------------------|
| (4)-----    | 50                          | 8                                      | 3.0                                        |
| (5)-----    | 20                          | 10                                     | 3.5                                        |
| (7)-----    | 40                          | 5                                      | 4.0                                        |
| (8)-----    | 40                          | 5                                      | 4.0                                        |
| (10)-----   | 40                          | 5                                      | 4.5                                        |
| (11)-----   | 40                          | 5                                      | 4.5                                        |
| (12)-----   | 50                          | 5                                      | 4.3                                        |
| (14)-----   | 40                          | 5                                      | 3.5                                        |
| (15)-----   | 40                          | 5                                      | 3.5                                        |
| (16)-----   | 50                          | 5                                      | 3.0                                        |
| (17)-----   | 30                          | 5                                      | 4.5                                        |
| (18)-----   | 30                          | 5                                      | 4.5                                        |
| (19)-----   | 30                          | 5                                      | 4.5                                        |
| (21)-----   | 40                          | 5                                      | 4.0                                        |
| (22)-----   | 40                          | 5                                      | 4.0                                        |
| (23)-----   | 40                          | 5                                      | 4.5                                        |
| (24)-----   | 60                          | 5                                      | 3.5                                        |
| (25)-----   | 50                          | 5                                      | 3.5                                        |
| (26)-----   | 60                          | 5                                      | 3.5                                        |

The compound of the Formula 20 can be prepared as follows:

18.5 parts of trichlorotriazine (cyanuric chloride) are dissolved in 40 parts of acetone and precipitated in a finely divided state with 100 parts of water and 100 parts of ice. 30.3 parts of 2-amino-naphthalene-4:8-disulfonic acid in the form of the neutral sodium salt and dissolved in 150 parts of water are then added. The mixture is stirred for a period of from 30 to 60 minutes at 0 to 4° C. and dilute sodium carbonate solution is added until the pH value remains constant at 5 to 6.5. No diazotizable amino compound must be detectable at the end of this period. To this primary condensation product are added 35 parts of 4:4'-diamino-diphenyl-2:2'-disulfonic acid that had been dissolved in 400 parts of water at 40° C. in the form of the sodium salt. The mixture is maintained for 1 hour at 40° C. and at a pH value of 6 to 7, the pH value being adjusted with sodium carbonate or sodium borate solution. The secondary condensation product can be obtained by salting out (that is, by the addition of 25 parts of sodium chloride per 100 parts by volume of the reaction mixture). The product is the compound shown by the Formula 20.

This product may then be further condensed at 40° C. with the primary condensation product described above to process the compound of the Formula 28.

The compounds of the Formulae 23 to 26 may be prepared by the above method when, instead of trichlorotriazine, equivalent proportions of 2-methoxy-4:6-dichloro-1:3:5-triazine, 3-methoxy-4:5:6-trichloropyridazine, 2:4:6-trichloropyrimidine or 4:5:6-trichloropyrimidine are used.

The other triazine compounds mentioned in these examples can likewise be prepared by methods in themselves known.

## EXAMPLE 2

A solution of 50 grams of silver nitrate in 450 milliliters of water is added during a period of 20 minutes at a temperature of 65° C. to a solution of 5 grams of gelatine, 42 grams of potassium bromide and 2.2 grams of potassium iodide in 450 milliliters of water. The mixture is allowed to mature for 15 minutes at 65° C. and is then cooled to 45° C. 20 milliliters of a 5% aqueous solution of the compound of the Formula 18 are added and the pH value is adjusted to 4.5 with citric acid. The silver halide along with the gelatine flocculates at once in the form of fine granules and settles out rapidly. After decanting the clear supernatant solution, the silver halide is redispersed in a solution of 80 grams of gelatine in 100 milliliters of water having a pH value of 7.2, and the emulsion is then allowed to mature to its optimum sensitivity in the conventional manner.

Solutions of the compounds listed in the following Table II may also be used in place of a solution of the compound of the Formula 18 in a process as described above.

35

TABLE II

| Formula No. | Amount, ml. of the solution | Concentration, percent of the solution | pH value at which flocculation is effected |
|-------------|-----------------------------|----------------------------------------|--------------------------------------------|
| 40          |                             |                                        |                                            |
| (4)-----    | 25                          | 8                                      | 3.0                                        |
| (5)-----    | 20                          | 10                                     | 3.5                                        |
| (7)-----    | 40                          | 5                                      | 4.0                                        |
| (8)-----    | 40                          | 5                                      | 3.5                                        |
| (11)-----   | 40                          | 5                                      | 5.0                                        |
| (17)-----   | 20                          | 5                                      | 4.5                                        |
| (19)-----   | 20                          | 5                                      | 4.5                                        |
| (20)-----   | 20                          | 5                                      | 4.5                                        |
| (21)-----   | 30                          | 5                                      | 4.0                                        |
| (22)-----   | 30                          | 5                                      | 4.0                                        |
| (24)-----   | 40                          | 5                                      | 3.5                                        |
| (25)-----   | 45                          | 5                                      | 3.5                                        |
| (26)-----   | 40                          | 5                                      | 4.0                                        |
| 50          |                             |                                        |                                            |

55 What is claimed is:

1. A process for the manufacture of a photographic silver halide emulsion by the flocculating method, which comprises flocculating the emulsion at a pH of 3 to 7, starting the emulsion to flocculate immediately after the first addition of flocculating agent, using as the flocculating agent a colorless compound containing
  - (a) at least one six-membered heterocyclic ring made up of 3 to 4 carbon atoms, at the most one halogen atom being bound to a carbon atom of said heterocyclic ring,
  - (b) at least one aromatic radical, and
  - (c) at least one acidic group imparting water-solubility to the compound, the emulsion starting to flocculate immediately on the addition of the flocculating agent and the adjustment of the pH to a value of 3 to 7.
2. A process according to claim 1 for the manufacture of a photographic silver halide emulsion by the flocculating method, which comprises flocculating the emulsion at a pH of 3 to 7, starting the emulsion to flocculate immediately after the first addition of flocculating agent, using

## 11

as the flocculating agent a colorless compound containing (a) at least one triazine radical, at the most one halogen atom being bound to a carbon atom of said triazine radical.

(b) at least one aromatic radical, and

(c) at least one acidic group imparting water-solubility to the compound and the adjustment of the pH to a value of 3 to 7.

3. A process according to claim 1 for the manufacture of a photographic silver halide emulsion by the flocculating method, which comprises flocculating the emulsion at a pH of 3 to 7, starting the emulsion to flocculate immediately after the first addition of flocculating agent, using as the flocculating agent a colorless compound containing

(a) at least one triazine radical, at the most one halogen atom being bound to a carbon atom of said triazine radical,

(b) at least one aromatic radical, and

(c) at least one sulfonic acid group and the adjustment of the pH to a value of 3 to 7.

4. A process according to claim 1 for the manufacture of a photographic silver halide emulsion by the flocculating method, which comprises flocculating the emulsion at pH of 3 to 7 using as the flocculating agent a colorless compound of the formula



wherein R<sub>1</sub> and R'<sub>1</sub> each contains at least one sulfonic acid group and represents a member selected from the group consisting of a benzene radical and a naphthalene radical and Y represents a halogen atom the emulsion

starting to flocculate immediately on the addition of the flocculating agent and the adjustment of the pH to a value of 3 to 7.

5. A process according to claim 1 for the manufacture of a photographic silver halide emulsion by the flocculating method which comprises flocculating the emulsion at a pH of 3 to 7 using as the flocculating agent a colorless compound of the formula



wherein R<sub>2</sub> and R'<sub>2</sub> each represents a naphthalene radical containing at least one sulfonic acid group, the emulsion starting to flocculate immediately on the addition of the flocculating agent and the adjustment of the pH to a value of 3 to 7.

## 12

6. A process according to claim 1 for the manufacture of a photographic silver halide emulsion by the flocculating method, which comprises flocculating the emulsion at a pH of 3 to 7 using as the flocculating agent a colorless compound of the formula



wherein R<sub>2</sub> and R<sub>3</sub> each represents a naphthalene radical containing at least one sulfonic acid group and Z represents a bridge member, the emulsion starting to flocculate immediately on the addition of the flocculating agent and the adjustment of the pH to a value of 3 to 7.

7. A process according to claim 1 for the manufacture of a photographic silver halide emulsion by the flocculating method, which comprises flocculating the emulsion at a pH of 3 to 5 using as the flocculating agent the compound of the formula



the emulsion starting to flocculate immediately on the addition of the flocculating agent and the adjustment of the pH to a value of 3 to 5.

8. A process according to claim 1 for the manufacture of a photographic silver halide emulsion by the flocculating method, which comprises flocculating the emulsion at a pH of 3 to 5 using as the flocculating agent the compound of the formula



the emulsion starting to flocculate immediately on the addition of the flocculating agent and the adjustment of the pH to a value of 3 to 5.

9. A process according to claim 1 for the manufacture of a photographic silver halide emulsion by the flocculating method, which comprises flocculating the emulsion at a pH of 3 to 5 using as the flocculating agent the compound of the formula



65 the emulsion starting to flocculate immediately on the addition of the flocculating agent and the adjustment of the pH to a value of 3 to 5.

## References Cited

- 70 UNITED STATES PATENTS
- 3,138,461 6/1964 Ryan ----- 96-94  
 3,288,775 11/1966 Anderau et al. ----- 96-111
- 75 J. TRAVIS BROWN, Acting Primary Examiner.